

## 1

3,008,868

DRAINAGE RATE OF CELLULOSIC  
PAPERMAKING SLURRIES

David A. Feigley, Jr., and Leonard N. Ray, Jr., Manor Township, Lancaster County, Pa., assignors to Armstrong Cork Company, Lancaster, Pa., a corporation of Pennsylvania  
No Drawing. Filed Dec. 23, 1957, Ser. No. 704,356  
16 Claims. (Cl. 162—179)

This invention relates generally to cellulosic fibrous sheets and more particularly to water-laid cellulosic fibrous sheets such as paper and felt. Still more particularly, the invention relates to the improvement in the drainage rate of cellulosic papermaking stocks.

In papermaking processes, it is always relatively simple to slow the drainage rate of a stock. This is most readily accomplished by mechanical refining of the fibers in a beater, Jordan engine, disc refiner, or the like. Increasing the drainage rate, however, is a more difficult problem. It is best accomplished by the beater saturation processes wherein the individual fibers in a papermaking stock are coated by depositing thereon a binder system which may be a rubber, resin, or other material. To state the difficulty another way, it is readily simple to adjust the Canadian freeness downward, but it is difficult to adjust the Canadian freeness upward.

A simplified flow diagram of the process is as follows:



It is the primary object of the present invention to present a process which will produce a dramatic decrease in the drainage time of a cellulosic papermaking stock without the necessity of coating the individual fibers with a substance such as a rubber which produces a sheet having vastly different properties from a sheet prepared from uncoated fibers. It is a further object of the present invention to present a process whereby a smoother sheet possessing greater flexibility and water resistance may be prepared in contrast with a sheet prepared by prior known processes.

These objects are accomplished in a surprisingly effective and straightforward manner. The invention contemplates improving the drainage rate of a cellulosic papermaking stock by treating the cellulosic fibers in the stock with a polyvalent metal ion selected from the group consisting of  $Al^{+++}$ ,  $Cr^{+++}$ ,  $Fe^{+++}$ . Subsequent to the polyvalent metal ion treatment, there is added to the stock a water-soluble salt of an organic, aliphatic, polycarboxylic acid containing at least 36 carbon atoms.

The cellulosic fibers contemplated for treatment by the present invention are those cellulosic fibers normally used in papermaking. As examples of such fibers, there

## 2

may be given sulfite pulp, kraft, soda pulp, cotton aids, cotton linters, rags, and newsprint. The stock is formed by known methods wherein the fibers are suspended in water to a workable consistency, using in the range of about 0.5-5%. Normally, a stock of the proper consistency is subjected to mechanical refinement until the desired degree of freeness is obtained. The precise freeness will be determined by the kind of paper or felt to be produced. Glassine papers, for example, call for the production of a stock with a Canadian freeness below 50 and usually above zero. Nonglassine papers call for a faster draining stock. The caliper or gauge of the paper or felt to be produced will also control to a large degree the freeness to which the stock is refined. In the present process, however, the freeness may be taken substantially below that which normally is needed to produce the particular sheet desired. Subsequent treatment to be described below will raise the freeness again to that needed to run the paper machine at normal speeds to produce the desired paper of the proper gauge. This feature of being able to take the stock to a lower freeness than that needed is responsible for the production of a smoother sheet having greater flexibility than would be obtainable if the lower freeness could not be used. Alternatively, the stock may be beaten or otherwise refined to the usual freeness. The subsequent treatment will raise the freeness above that which normally must be used and will thus allow an increase of machine speed or the production of a thicker sheet. It will be apparent that this control of the stock freeness can be carried out in varying degrees.

The cellulosic fibers in the stock are then treated with either aluminum, iron, or chromium ion in the trivalent state. Such treatment may be accomplished by the mere addition of an aluminum, ferric, or chromic salt to the stock. Mixtures thereof can be used. Preferably, however, the salt is taken up in water and added to the stock in the form of a solution. The addition of a solution expedites the distribution of the metallic ion throughout the water phase of the stock and eliminates the need for waiting for the salt to dissolve in the water phase of the stock itself.

The amount of metallic ion to be added to the stock need not be large. As a general rule, about 0.1% by weight of the metal based on the dry weight of the fibers being treated is ample to render the fibers amenable to subsequent reaction with the organic acid salt. Stated another way, the metallic salt should be added in an amount of about 1-5% by weight of the salt based on the dry weight of the fibers being treated. Such amounts of the salt will always supply sufficient ion to successfully pretreat the cellulosic fibers. Larger amounts of the salt above that amount stated will do no actual harm to the stock. However, in the interest of avoiding waste of the metallic salt, it is preferred that the amount of the salt be kept within the stated range of 1-5% by weight of the salt based on the dry weight of the fibers. If too large an amount of the salt is introduced into the stock, an insoluble soap may be formed on subsequent addition of the organic acid salt. This situation will produce a further waste of the acid and, from this standpoint, is undesirable.

Any salt of aluminum, iron, or chromium may be used so long as the salt is reasonably soluble in water and the metal is in the trivalent state. The nitrate, sulfate, and chloride are the commonest soluble salts of aluminum, iron, and chromium. Papermakers' alum is the salt of choice.

Although the metallic ion has been described as added to the slurry subsequent to the mechanical refining step, such point of addition is not critical. Actually the metallic ion in the form of a salt may be added to the stock

at any time during the formation of the stock. Thus it may be added prior to the time at which the stock is mechanically refined. If this be done, the stock will be ready for the addition of the polycarboxylic acid salt as soon as the proper degree of refinement has been obtained.

Following treatment of the stock with the polyvalent metal ion, the cellulosic fibers are then in condition to be reacted with the organic acid salt.

The acids suitable for use in the present invention are best illustrated by the dimerized and trimerized fatty acids which are readily available in commerce. These acids are prepared by the thermal polymerization of drying oil acids carried out in a pressure vessel in the presence of water in the form of steam. The resulting compositions generally contain on the average of about 3% monomer, 75% dimer, and 22% trimer. Such a product is known as dimerized fatty acid and will have an iodine value of approximately 90 and an acid number of approximately 190. The dimerized acid itself is essentially a 36-carbon dicarboxylic acid obtained by dimerization of the linoleic acid of soya, cottonseed, corn, and linseed oils of commerce; it possesses olefinic unsaturation. The product is frequently referred to as dilinoleic acid. This dimerized acid product may be purchased under the name "Empol 1022." It is apparent that the dimerized acids and the trimerized acids resulting from the above-described pressurized process may be separated or further concentrated as desired. Thus the trimer acid may be purchased as such. The trimer acid is 54-carbon acid and contains a plurality of carboxylic acid groups. As a further variation on the dimer and trimer acids, any residual olefinic unsaturation in the carbon chain may be eliminated by hydrogenation. The hydrogenated dimer acid may be purchased under the name "Emery 3020-S"; the predominantly straight trimer acid may be purchased under the name "Emery 3055-S." In addition to the above-described acids themselves, there may also be used the maleic acid or maleic anhydride adducts (Diels-Alder reaction) of any of the unsaturated acids described above.

The organic acids useful in the present invention must be converted to their water-soluble forms. In view of the size of most of the molecules, the compounds are not generally *per se* soluble. They are, however, easily rendered soluble by reaction with an alkaline material, such as ammonia, sodium hydroxide, potassium hydroxide, carbonates of ammonia, sodium and potassium and even to some extent with alkaline earth metal compounds and organic amines. It must be emphasized that the compounds used in the present invention need not be very soluble to be operable. The compounds are used in relatively small amounts compared with the amount of water present, so easy solubility is not necessary. In the present specification and claims, it is contemplated that the defined organic polycarboxylic acids are rendered water-soluble where necessary by reaction of the acid with a solubilizing alkaline ingredient to form a salt. Thus the compound to be used will be selected from the group consisting of water-soluble polycarboxylic acids, water-soluble polycarboxylic acid salts, and mixtures thereof.

As is the case with the metallic salt, the polycarboxylic acid salt need not be added in large amounts. Amounts of the polycarboxylic acid salt in the range of about 1-5% by weight polycarboxylic acid based on the dry weight of the cellulosic fibers is the broad range, with the preferred amount running about 3% by weight acid based on the weight of the fibers. Amounts smaller than about 1% by weight do not bring about a significant improvement in the drainage rate, while amounts larger than about 5% by weight are generally wasted since the excess simply remains in the white water.

The actual step of adding the organic polycarboxylic acid salt to the stock is readily accomplished by simply physically adding the salt to the slurry. Preferably the salt will first be taken up in water to form an aqueous

5 solution or suspension and the salt will be added in the form of that solution or suspension. Use of a solution aids in quick dispersion of the water-soluble polycarboxylic acid throughout the stock and hastens the reaction that takes place between the polycarboxylic acid and the surface of the cellulosic fibers. Once the polycarboxylic acid salt has been added to the stock, preferably with gentle agitation, reaction will be complete normally within 15 minutes and usually within about 5 minutes. The freeness of the stock as compared with identical untreated stock will be found to have increased as much as 70%. Stated another way, the rate of drainage of the stock will be found to be about half that of identical untreated stock, and frequently the drainage time will be reduced to appreciably less than half of that of the untreated stock.

10 The reason for the improved drainage rate obtained by the present invention is not clearly understood. It is postulated that the addition of the polyvalent metal ion brings about a reversal of the charge carried by the cellulosic fibers in water suspension. This charge reversal allows the treated fibers to react with the water-soluble polycarboxylic acid to produce a fiber having a modified surface, which modified surface apparently brings about the improved drainage rate. It is to be noted that mere treatment of the cellulosic fibers in water suspension with the polyvalent metal ions does not change the drainage characteristics of the stock significantly. An attempt to react the cellulosic fibers with polycarboxylic 15 acids salts without prior treatment with polyvalent metallic ions does not produce any change in the drainage characteristics of the stock. Furthermore, treatment of the cellulosic fibers with aluminum, ferric, or chromic ion followed by an attempt to react the treated fibers with an organic acid containing less than 36 carbon atoms will produce a stock having drainage characteristics substantially worse than that of the dimer soap-treated stock.

20 Stocks treated by the present invention may then be handled as any other papermaking stock in the production of useful products such as various papers and felts. Papers produced by the present process possess increased 25 flexibility and hence increased resistance to breakage and tearage when compared with similar papers prepared by means in which the present invention has not been used.

30 The usual sizing agents such as starch, casein, and cellulose drums may be used in conjunction with the sheet-making processes described herein. Sizing and other processing variables may be carried out after the fibers have been treated and before the treated slurry is passed to the wire, or once the sheet has been formed on the wire. For certain purposes it may be desirable to precipitate synthetic rubber binder onto the cellulosic 35 fibers to strengthen the sheet. Small amounts, generally 1-5% by weight rubber based on the weight of the fibers, will usually suffice for this purpose. Mere addition of the latex to the treated stock followed by agitation will cause precipitation of this small amount of rubber onto the fibers. Where larger amounts of rubber are to be added, addition of a precipitating agent, such as a solution of papermakers' alum, will speed and complete the 40 rubber precipitation. The synthetic rubbers which can be used are those used in beater saturation processes and include butadiene-styrene copolymers, butadiene-acrylonitrile copolymers, polychloroprene, and the like.

45 The following examples illustrate several embodiments of the invention. All parts are by weight unless otherwise stated.

#### Example 1

50 Into 4,000 parts of water is placed 40 parts sulfite pulp and the stock is beaten in a laboratory beater for 15 minutes. The Canadian 3-gram freeness of the resulting stock is 370 cc. and the drainage time in a 12" x 12" laboratory sheet mold is 29 seconds.

55 To a stock prepared exactly as described above, there is added one part papermakers' alum dissolved in 50

parts of water, with gentle agitation. There is then added a soap solution sufficient to supply 1.5 parts of a hydrogenated dimer acid (hydrogenated dilinoleic acid, "Emery 3020-S"). The soap solution is prepared by placing the 1.5 parts of the dimer acid into 50 parts of water and adding sufficient potassium hydroxide to dissolve the acid.

The Canadian 3-grams freeness of the treated stock was 570 cc. and the drainage time in the laboratory 12" x 12" sheet mold was 13 seconds. The resulting sheet was dried in an air circulating oven maintained at 195° F. and proved to be smoother than an identical sheet made from stock not treated with the metallic ion and polycarboxylic acid soap. The sheet also was significantly more flexible and possessed greater water resistance than an untreated sheet.

#### Example II

Example I was repeated save that in place of the alum solution there was used a solution of ferric chloride prepared by dissolving one part of the salt,  $\text{FeCl}_3 \cdot 6\text{H}_2\text{O}$ , in 100 parts water. After the soap treatment the stock had a Canadian freeness of 480.

#### Example III

Example I is repeated except that the potassium salt of a predominantly straight trimer acid (Emery 3055-S) was used. The resulting stock has a Canadian freeness of 510.

#### Example IV

Example I is repeated with cotton aids as the cellulosic fiber and the potassium soap of dimerized acid (Empol 1022) as the organic salt. The untreated stock has a Canadian freeness of 300 cc., whereas the treated stock has a Canadian freeness of 550 cc.

#### Example V

Example I is repeated using newsprint as the cellulosic fiber. An improvement in Canadian freeness from 250 to 420 is noted.

We claim:

1. In a papermaking process wherein a stock comprising papermaking cellulosic fibers suspended in water is formed into a sheet on a papermaking machine, the improved process of improving the drainage rate of said stock which comprises treating said cellulosic fibers in said stock with a polyvalent metal ion selected from the group consisting of  $\text{Al}^{+++}$ ,  $\text{Cr}^{+++}$ , and  $\text{Fe}^{+++}$ , and adding to the treated stock a water-soluble salt of an organic, aliphatic, polycarboxylic, polymerized fatty acid containing at least 36 carbon atoms.

2. A process according to claim 1 wherein said metal ion is aluminum.

3. A process according to claim 1 wherein said polycarboxylic acid is a saturated acid.

4. A process according to claim 1 wherein said polycarboxylic acid is an unsaturated acid.

5. A process according to claim 1 wherein said polycarboxylic acid is added in amount of about 1-5% by weight acid based on the dry weight of said cellulosic fibers.
6. A method according to claim 1 wherein said polycarboxylic acid comprises dilinoleic acid.
7. A process according to claim 1 wherein said polycarboxylic acid contains 54 carbon atoms.
8. A process according to claim 1 wherein said water-soluble salt of an organic polycarboxylic acid comprises the potassium salt.
9. A process of forming a sheet which comprises forming in water a slurry of cellulosic fibers, treating said cellulosic fibers with a polyvalent metal ion selected from the group consisting of  $\text{Al}^{+++}$ ,  $\text{Cr}^{+++}$ , and  $\text{Fe}^{+++}$ , adding to the treated slurry a water-soluble salt of an organic, aliphatic, polycarboxylic, polymerized fatty acid containing at least 36 carbon atoms, and forming a sheet from the thus treated slurry.
10. The process according to claim 9 wherein said polyvalent metal ion comprises aluminum and said water-soluble salt of a polycarboxylic acid comprises the potassium salt of hydrogenated dilinoleic acid.
11. A water-laid sheet comprising cellulosic fibers whose surfaces are reacted with an organic, aliphatic, polycarboxylic, polymerized fatty acid containing at least 36 carbon atoms.
12. A sheet according to claim 11 wherein said polycarboxylic acid contains 54 carbon atoms.
13. A sheet according to claim 11 wherein said polycarboxylic acid comprises a saturated acid.
14. A sheet according to claim 11 wherein said polycarboxylic acid comprises an unsaturated acid.
15. A sheet according to claim 11 wherein the surfaces of said cellulosic fibers are reacted with about 1-5% by weight of said polycarboxylic acid based on the total weight of said fibers.
16. A sheet according to claim 11 wherein said polycarboxylic acid comprises dilinoleic acid.

#### References Cited in the file of this patent

#### UNITED STATES PATENTS

|    |           |                  |               |
|----|-----------|------------------|---------------|
| 45 | 1,958,202 | Novak            | May 8, 1934   |
|    | 2,447,064 | Gebhart et al.   | Aug. 17, 1948 |
|    | 2,473,798 | Kienle et al.    | June 2, 1949  |
|    | 2,665,206 | Bradley          | Jan. 5, 1954  |
|    | 2,665,207 | McMillan et al.  | Jan. 5, 1954  |
| 50 | 2,666,699 | McQuiston et al. | Jan. 19, 1954 |
|    | 2,731,481 | Harrison et al.  | Jan. 17, 1956 |
|    | 2,772,970 | Feigley          | Dec. 4, 1956  |
|    | 2,812,342 | Peters           | Nov. 5, 1957  |
| 55 | 2,887,431 | Piersol          | May 19, 1959  |
|    | 2,930,106 | Wrotnowski       | Mar. 29, 1960 |
|    | 2,940,892 | Feigley et al.   | June 14, 1960 |

UNITED STATES PATENT OFFICE  
CERTIFICATION OF CORRECTION

Patent No. 3,008,868

November 14, 1961

David A. Feigley, Jr., et al.

It is hereby certified that error appears in the above numbered patent requiring correction and that the said Letters Patent should read as corrected below.

Column 1, line 61, for "accomplished" read -- accomplished --; column 2, line 11, for "above" read -- about --; same line 11, strike out "papers", second occurrence; column 5, line 8, for "3-grams" read -- 3-gram --.

Signed and sealed this 24th day of April 1962.

(SEAL)

Attest:

ESTON G. JOHNSON  
Attesting Officer

DAVID L. LADD  
Commissioner of Patents